

# United States Patent [19]

Niebylski et al.

[11] 3,847,591

[45] Nov. 12, 1974

[54] **LEAD-ZINC FOAMS**

[75] Inventors: **Leonard M. Niebylski, Birmingham; Chester P. Jarema, Detroit, both of Mich.**

[73] Assignee: **Ethyl Corporation, Richmond, Va.**

[22] Filed: **Nov. 1, 1973**

[21] Appl. No.: **411,893**

**Related U.S. Application Data**

[63] Continuation-in-part of Ser. No. 155,210, June 21, 1971, Pat. No. 3,790,365, which is a continuation-in-part of Ser. No. 879,915, Nov. 24, 1969, abandoned.

[52] U.S. Cl..... **75/20 F, 164/79**

[51] Int. Cl..... **B22d 27/00**

[58] **Field of Search** ..... **75/20 F, 29 R; 164/79**

[56] **References Cited**

**UNITED STATES PATENTS**

3,214,265 10/1965 Fiedler ..... **75/20 F**

|           |         |                     |                 |
|-----------|---------|---------------------|-----------------|
| 3,305,902 | 2/1967  | Bjorksten .....     | <b>75/20 UX</b> |
| 3,705,030 | 12/1972 | Berry et al.....    | <b>75/20 F</b>  |
| 3,816,952 | 6/1974  | Niebyski et al..... | <b>75/20 F</b>  |

**FOREIGN PATENTS OR APPLICATIONS**

724,090 12/1965 Canada..... **75/20 F**

*Primary Examiner*—Andrew R. Juhasz

*Assistant Examiner*—V. K. Rising

*Attorney, Agent, or Firm*—Donald L. Johnson; Robert A. Linn

[57]

**ABSTRACT**

Good quality lead foams are made if the lead is alloyed with zinc, the mixture is treated with CO<sub>2</sub> prior to foaming, titanium hydride is used as the foaming agent, the foam is rapidly cooled after formation, and a shallow mold is used. The alloy-hydride mixture can be solidified prior to foaming.

**1 Claim, No Drawings**

## LEAD-ZINC FOAMS

## CROSS-REFERENCE TO RELATED APPLICATIONS

This is a continuation-in-part of application Ser. No. 155,210 now U.S. Pat. No. 3,790,365, issued Feb. 5, 1974, filed June 21, 1971, which in turn is a continuation-in-part of application Ser. No. 879,915, filed Nov. 24, 1969, and now abandoned.

## BACKGROUND OF THE INVENTION

Lead-zinc alloy has been foamed, and U.S. Pat. Nos. 2,937,938 and 3,305,902 refer to foaming various metals and alloys thereof. In these disclosures zinc and lead are among the metals mentioned.

Use of carbon dioxide to thicken metal prior to foaming is disclosed in Canadian Pat. No. 912,283.

## SUMMARY OF THE INVENTION

A preferred embodiment is a process for preparing a foam of a lead-based alloy, said alloy having from about 1.5 weight per cent to about 5 weight per cent zinc, said process comprising substantially saturating a molten mass of said alloy with  $\text{CO}_2$ , adding with stirring from about 2 g to about 5 g of  $\text{TiH}_2$  per 100 gram portion of lead while maintaining the temperature of the mass to be foamed below about 410°C., subsequently raising the temperature to from about 420°C. to about 475°C. to foam said mass, and then quickly cooling the foam thereby produced below its solidification temperature.

## DESCRIPTION OF PREFERRED EMBODIMENTS

Preferably the lead contains from about 1 weight per cent to about 10 weight per cent or higher, and more preferably from about 1.5 weight per cent to about 6 weight per cent zinc. In a preferred embodiment the metal mass consists essentially of lead and zinc and has from 1.5 to 5 weight per cent zinc.

Treatment of the metal mass with  $\text{CO}_2$  prior to foaming improves the foam quality. Solid carbon dioxide can be used. Best results are obtained if the molten mass is saturated or substantially saturated with  $\text{CO}_2$  prior to foaming.

The molten metal to be foamed can be at about 475°-525°C. prior to initiation of  $\text{CO}_2$  addition. This temperature range isn't critical since any temperature from the solidification temperature to the boiling point can be used. Preferably, the  $\text{CO}_2$  is added as solid  $\text{CO}_2$ , but gaseous  $\text{CO}_2$  can be used as well. Addition of solid  $\text{CO}_2$  can appreciably lower the metal temperature. Thus, we add  $\text{CO}_2$  at a rate at which solidification doesn't take place. Any convenient rate which avoids solidification can be used.

The time of  $\text{CO}_2$  addition isn't critical; and usually is complete in from one-half minute to 5 minutes. To some extent, the time depends on size of the mass to be foamed. Stirring while adding assists uniform mixing of  $\text{CO}_2$  and metal and is preferred. Other means of agitation can be used.

If  $\text{CO}_2$  is added until the metal is saturated or nearly so, and at a temperature above the foaming temperature, the melt can be saturated or substantially saturated with  $\text{CO}_2$  at foaming temperature. The amount of foaming agent used depends in part on the density of foam desired. Of the hydride foaming agents,  $\text{TiH}_2$  is

preferred. For each 100 gram portion of lead to be foamed, preferably from about 2 to about 5 grams, more preferably from 3 to 5 grams of  $\text{TiH}_2$  is used. In a preferred embodiment, for foams of about 10 per cent density, from 4.5 to 5 grams (per 100 gram portion of lead) is employed.

The hydride is added to the molten metal mass at a temperature below about 410°C. Preferably the mixture is at about 400°C. when the hydride is added.

10 Stirring or other means of agitation which enhances mixing of the hydride in the metal mass are preferentially used when adding the foaming agent.

15 After introducing the hydride into the mass to be foamed, the mass temperature is raised to a foaming temperature of from about 420°C. to about 475°C. This decomposes the foaming agent and foams the metal.

20 After the desired degree of foaming has been reached, the foamed mass is quickly cooled. This can be accomplished by quenching with tap water, or with dry ice, or with a chilled copper plate heat sink, or other similar technique.

25 Conducting the foaming in a shallow vessel, say up to about 5 inches in height, enhances the ability to rapidly cool the foam. Thus, this expedient is preferred.

## EXAMPLE

30 A procedure for producing a high quality foam is as follows:

35 Add 5 per cent zinc to chemically pure Pb; raise the melt temperature to 500°C. and add  $\text{CO}_2$  (dry ice) until no more  $\text{CO}_2$  can be added. Then at 400°C., add approximately 5 g  $\text{TiH}_2$ /100 g Pb with vigorous stirring. Cast into a preheated mold (470°C.) and place in an oven at that temperature for 3-5 minutes. After that time, the Pb foam is quenched in the oven with dry ice or  $\text{H}_2\text{O}$  before moving so as to prevent any foam drainage or collapse.

40 Similar results are obtained when the amount of zinc is from 1.5 to 5.0 per cent, the  $\text{CO}_2$  is added at from 475° to 525°C., the  $\text{TiH}_2$  is added at from 400° to 410°C., the amount of  $\text{TiH}_2$  is from 2 to 5 g per 100 g of lead, the foaming temperature is from 420° to 475°C., and the foaming time is from 5 to 30 minutes.

50 Lead Foam Strength — Compressive strength tests were run on lead foams which had been made. Sample size varied from 1 inch  $\times$  1 inch  $\times$  0.75 inch to 2 inches  $\times$  0.75 inch. The following data were obtained:

| Sample No. | Density (pcf) | Compressive Strength (psi) |   |
|------------|---------------|----------------------------|---|
|            |               | 1                          | 2 |
| 60         | 68.7          | 38.1                       |   |
|            | 80.6          | 44.2                       |   |
|            | 96.5          | 100.9                      |   |
|            | 101.3         | 70.0                       |   |
|            | 97.3          | 65.0                       |   |
|            | 97.9          | 105.0                      |   |
|            | 98.0          | 135.0                      |   |

65 All compressive values were taken at 10 per cent compression of the 0.75 inch thickness. There was no

peaking in the load-deflection curve, only a change in slope at about 5 per cent compression. The Pb samples showed no crumbling at up to 30 per cent compression.

The data shows that the lead foams have strengths of 0.5-1.5 psi/lb of foam. However, when compared to the strength/weight ratio of solid lead which is 2.5 psi/lb, the foam strengths are appreciable.

We have shown the feasibility of producing a foamable lead-hydride alloy which can be made into a foam by simply heating it in a furnace. In this work,  $TiH_2$  is mixed into Pb-5 per cent zinc alloy after  $CO_2$  treatment and below 400°C. The mixture is then poured into a mold and solidified. Later it is placed in an oven at 470°C. where, after a few minutes, the metal will foam.

Good quality foams have been produced having little or no drainage.

Tests have been conducted to show feasibility of use of a lead foam produced by the process of the above example as an acoustical material for sound deadening, dampening or isolation purposes. Measurements were made in a Brüel and Kjaer acoustic tube on a 9.4 cm specimen at 250, 500, 1,000 and 2,000 Hz. The specimens were backed by a steel plate. The method of measurement is that described in the American Society for Testing and Materials Standard Method of Test for Impedance and Absorption of Acoustical Materials by the Tube Method, ASTM Designation C384-58.

#### Results of Test

The  $\alpha_n$ 's are the absorption coefficients at normal incidence. They mean the fraction of the incident sound power absorbed when sound impinges perpendicularly on the material. The  $\alpha_a$ 's are approximate coefficients which might be obtained by a large scale test in the reverberation room where sound impinges on the material at all angles.

|    |                          | Hz   | Normal Coefficients, $\alpha_n$ | Approximate Random Coefficients, $\alpha_a$ |
|----|--------------------------|------|---------------------------------|---------------------------------------------|
| 5  | Foamed Pb-5 per cent     | 250  | .09                             | .17                                         |
|    |                          | 500  | .15                             | .28                                         |
|    | Zn Alloy                 | 1000 | .19                             | .34                                         |
|    |                          | 2000 | .06                             | .12                                         |
| 10 | Lead Sheet-Urethane Foam | 250  | .05                             | .11                                         |
|    |                          | 500  | .04                             | .05                                         |
|    |                          | 1000 | .04                             | .05                                         |
|    | Composite                | 2000 | .07                             | .13                                         |

These data indicate foamed lead is better than the sheet lead-urethane foam composite in the range 500-1,000 Hz whereas the materials are nearly equal in absorption at the high and low frequency ranges. Similar results are obtained on foams having a density from 68 to 101 pcf.

The sheet lead-urethane foam composite used in the above test for comparison was a commercially available acoustical material.

If desired, the foams of this invention can be bonded to urethane or Polyvinyl chloride foams to form an acoustical composite.

The foams of this invention can be used as shock absorbing materials in passenger or freight compartments of vehicles to prevent or lessen damage on impact.

We claim:

1. Process for preparing a metal foam from a lead based metal having from 1.5 to 5 weight per cent zinc, 30 said process comprising substantially saturating a molten mass of said metal with  $CO_2$ , subsequently adding with stirring from 1.5 to 5 grams of  $TiH_2$  per 100 gram portion of Pb while maintaining the temperature of the mass below about 410°C., subsequently raising the temperature to from about 420°C. to about 475°C. to foam said mass, and quickly cooling the foam thereby produced below its solidification temperature to form a set cellular product.

\* \* \* \* \*